

## UNITED STATES PATENT OFFICE

2,238,631

## YELLOW FOG INHIBITOR FOR PHOTOGRAPHIC MATERIAL

Fritz Dersch and Newton Heimbach, Binghamton, N. Y., assignors, by mesne assignments, to General Aniline & Film Corporation, New York, N. Y., a corporation of Delaware

No Drawing. Application May 4, 1939,  
Serial No. 271,720

11 Claims.

(Cl. 95—7)

Our invention relates to photographic materials containing anti-yellow fogging agents, and more particularly to the use of sulfonium iodides and related compounds as such agents.

It is well known that many light sensitive emulsions, such as gelatine-silver halide emulsions, have a tendency to fog. There are two general types of this fog: first, ordinary grey fog such as is caused by premature exposure, by excessive ripening of the emulsion, or by ordinary aging of the emulsion; and, secondly, so-called yellow fog, color fog, or dichroic fog. This yellow fog is essentially a colloidal deposit of silver, of which the great degree of subdivision or minute particle size chiefly determines the color intensity and general appearance. The fog is usually predominantly yellow and is most apparent in the lighter portions of a negative. The colloidal particles of silver may, however, appear green by reflected light and yellow or red by transmitted light, which effect is often referred to as color fog or dichroic fog.

Yellow fog may be caused by the emulsion itself or one of its constituents, or by some factor in the preparation of the emulsion. It may also result from a variety of conditions in connection with the processing of the film. For example, the presence of traces of fixing solution or of excess silver halide solvent such as sulfite in the developing bath, or the use of nearly exhausted developing or fixing baths, will commonly cause yellow fog. The problem is especially prevalent in the processing of X-ray films, where thick emulsions and the repeated use of partially exhausted fixing solutions contribute to the production of yellow fog.

Other possible causes of yellow fog have been described in the literature pertaining to this art, and various remedies have been suggested. For example, United States Patent No. 2,059,642 suggests the use of a mixture of soluble gold and mercury salts to prevent both grey and yellow fog. Likewise, German Patent No. 635,605 (1936) and Photographische Korrespondenz, Band 72, Seite 148, disclose the use of diphenyliodonium salts in emulsions and in developing, washing or fixing baths as tending to prevent yellow fog. Cassell's Cyclopaedia of Photography, 1912, vol. 1, p. 266, also recommends treatment with a bath of sodium sulfite and potassium cyanide to remove the yellow fog once it has formed. These methods cannot be considered wholly satisfactory, since they often lead to such disadvantages as gradation loss, formation of grey fog, or loss

of sensitivity. One object of our invention is to provide a new class of fog inhibiting agents which tend to prevent the formation of yellow fog in photographic materials while avoiding the difficulties and defects of the prior art procedures.

Another object is to provide anti-yellow fog agents which may be incorporated in a photographic emulsion or in a surface or substratum layer without noticeably decreasing the sensitivity of the emulsion.

A still further object is to provide new yellow fog inhibitors which may be incorporated in the developing bath itself or in a separate processing bath.

15 Still another object is the treatment of gelatines which normally cause yellow fog when used in photographic emulsions with compounds which decrease this yellow fogging tendency.

Further objects and advantages will appear 20 from the following specification.

We have found that the above objects are accomplished by the use of sulfonium iodides and the related selenium and tellurium compounds as well as the addition products or salts of the 25 above compounds with various metal and alkyl iodides, as yellow fog inhibitors.

These compounds all contain the grouping



30 wherein Y is sulfur, selenium, or tellurium, and I represents iodine. While we do not wish to limit ourselves to any particular theory, it is our belief based on experience that the feature responsible for the desirable results produced by these compounds is the tetravalent Y grouping, one valence of which is "taken up" by an iodine atom. Accordingly it is immaterial how the 35 three other valences of the "Y atom" are supplied, so long as they are supplied by organic radicles. Thus our invention includes compounds of the general formulae:



45 and 50 wherein Y is sulfur, selenium, or tellurium as above, and wherein the substituents R<sub>1</sub>, R<sub>2</sub> and

$R_3$  may be substituted or unsubstituted alkyl, cycloalkyl, aryl, aralkyl, or heterocyclic groups and may be like or unlike, and wherein



is a heterocyclic grouping.

Typical compounds having these desirable properties thus include: alkyl sulfonium-, selenonium-, and telluronium iodides such as trimethyl sulfonium iodide, triethyl sulfonium iodide, and methyl diethyl sulfonium iodide; alkyl-cycloalkyl sulfonium-, selenonium- and telluronium iodides, such as dimethyl cyclohexyl sulfonium iodide; substituted aryl sulfonium-, selenonium-, and telluronium iodides, for example, phenyl-bis-(p-bromophenyl)- sulfonium iodide



alkyl-aryl sulfonium-, selenonium-, and telluronium iodides, for instance methyl diphenyl telluronium iodide



alkyl-aralkyl sulfonium-, selenonium-, and telluronium iodides, such as methyl dibenzyl sulfonium iodide



heterocyclic sulfonium-, selenonium- and telluronium iodides, for example methyl tetramethylene sulfonium iodide



and phenyl thio-o-diphenylene sulfonium iodide



and finally, addition products or salts of any of the above compounds with various metal and alkyl iodides, for instance with cadmium iodide, mercuric iodide, bismuth iodide, and iodoform. Typical examples of such addition products are:



In order that those skilled in the art may

better understand the nature and scope of this invention, the following specific examples are given without any intention of limiting the invention thereto.

#### Example 1

To 500 g. of a light sensitive gelatino-silver halide emulsion which normally shows yellow fog, melted at 40° C., are added from 10 to 20 mg. of trimethyl sulfonium iodide. The mixture is coated on a suitable support, chilled, and dried in the customary manner. The emulsion thus treated is free from yellow fog.

#### Example 2

The trimethyl sulfonium iodide of the preceding example may be applied to the emulsion by including it in a surface coating. In such a case the amount used should be so chosen that the same concentration of sulfonium iodide per unit area of coated film based on relative thickness of surface and emulsion coatings, is obtained as in Example 1. Thus, if the surface coating is one-tenth the thickness of the emulsion coating, approximately ten times as much trimethyl sulfonium iodide, or from 100 to 200 mg., is added to 500 g. of surface coating solution. The film having a surface coating thus treated is free from yellow fog.

#### Example 3

To one liter of a common developer solution, such as any standard metol - hydroquinone formula, is added 20 to 30 mg. of triethyl sulfonium iodide. A film having an emulsion which normally exhibits a tendency to form yellow fog may be developed in this solution without the formation of such fog.

#### Example 4

To 500 g. of a light sensitive gelatino-silver halide emulsion as in Example 1, melted at 40° C., are added from 10 to 20 mg. of phenyl thio-o-diphenylene sulfonium iodide. The mixture is coated on a suitable support, chilled and dried in the usual way. The emulsion thus treated is free from yellow fog.

#### Example 5

To 500 g. of a light sensitive gelatino-silver halide emulsion as in Example 1, melted at 40° C., are added from 10 to 20 mg. of triethyl selenonium iodide. The mixture is coated on a suitable support, chilled and dried in the usual way. The emulsion thus treated is free from yellow fog.

#### Example 6

To 500 g. of a light sensitive gelatino-silver halide emulsion as in Example 1, melted at 40° C., are added from 10 to 20 mg. of triethyl sulfonium iodide. The mixture is coated on a suitable support, chilled and dried in the usual way. The emulsion thus treated is free from yellow fog.

The quantities of the compounds used may, of course, be varied slightly to suit the particular conditions involved.

Since the presence of these new compounds tends to prevent yellow fog whether they are incorporated directly into the emulsion, added to a separate surface or substratum layer, added to the developing bath, or used in a separate processing bath, we have used the term "photographic material" in the appended claims in a broad sense as including each of these possible applications.

We claim:

1. A photographic material containing as a yellow fog inhibitor for silver halide emulsions an organic compound having the grouping



wherein Y is a tetravalent atom selected from the group consisting of sulfur, selenium, and tellurium and wherein the dangling valences are supplied by organic radicles.

2. A photographic material containing as a yellow fog inhibitor for silver halide emulsions an organic compound having the grouping



and wherein the dangling valences are supplied by organic radicles.

3. A photographic material containing as a yellow fog inhibitor for silver halide emulsions an organic substance corresponding to the formula



wherein Y is a tetravalent atom selected from the group consisting of sulfur, selenium, and tellurium and wherein the dangling valances are supplied by organic radicles.

4. A photographic material containing as a yellow fog inhibitor for silver halide emulsions a substance corresponding to the formula



wherein Y is a tetravalent atom selected from the group consisting of sulfur, selenium, and tellurium.



is a heterocyclic group and R3 is a member selected from the group consisting of substituted and unsubstituted alkyl, cycloalkyl, aryl, aralkyl, and heterocyclic groups.

5. A photographic material containing as a

yellow fog inhibitor for silver halide emulsions a substance corresponding to the formula



wherein



is a heterocyclic group, and R3 is a member selected from the group consisting of substituted and unsubstituted alkyl, cycloalkyl, aryl, aralkyl, and heterocyclic groups.

6. A photographic material containing as a yellow fog inhibitor for silver halide emulsions a substance corresponding to the formula



wherein Y is a tetravalent atom selected from the group consisting of sulfur, selenium, and tellurium, and wherein R1, R2 and R3 represent alkyl groups.

7. A photographic material containing as a yellow fog inhibitor for silver halide emulsions a substance corresponding to the formula



35 wherein R1, R2 and R3 represent alkyl groups.

8. A photographic material containing trimethyl sulfonium iodide as a yellow fog inhibitor for silver halide emulsions.

9. A light sensitive photographic gelatino-silver halide emulsion containing from 10 to 20 mg. of trimethyl sulfonium iodide per 500 g. of emulsion as a yellow fog inhibitor.

10. A photographic material containing triethyl sulfonium iodide as a yellow fog inhibitor for silver halide emulsions.

11. A light sensitive photographic gelatino-silver halide emulsion containing from 10 to 20 mg. of triethyl sulfonium iodide per 500 g. of emulsion, as a yellow fog inhibitor.

FRITZ DERSCH.  
NEWTON HEIMBACH.